



US005893953A

# United States Patent [19]

## Bhargava

[11] Patent Number: 5,893,953  
[45] Date of Patent: Apr. 13, 1999

[54] COPPER ALLOY AND PROCESS FOR OBTAINING SAME

[75] Inventor: **Ashok K. Bhargava**, Cheshire, Conn.

[73] Assignee: **Waterbury Rolling Mills, Inc.**, Waterbury, Conn.

[21] Appl. No.: **08/931,696**

[22] Filed: **Sep. 16, 1997**

[51] Int. Cl. <sup>6</sup> ..... C22C 1/08

[52] U.S. Cl. ..... 148/685; 148/680

[58] Field of Search ..... 148/680, 684, 148/685

### [56] References Cited

#### U.S. PATENT DOCUMENTS

|           |         |                  |         |
|-----------|---------|------------------|---------|
| 2,062,427 | 12/1936 | Pierson          | .       |
| 3,923,558 | 12/1975 | Shapiro et al.   | 148/412 |
| 4,586,967 | 5/1986  | Shapiro et al.   | 420/472 |
| 4,605,532 | 8/1986  | Knorr et al.     | 420/472 |
| 4,627,960 | 12/1986 | Nakajima et al.  | 420/472 |
| 4,666,667 | 5/1987  | Kamio et al.     | 420/471 |
| 4,822,562 | 4/1989  | Miyafuji et al.  | 420/472 |
| 4,935,076 | 6/1990  | Yamaguchi et al. | 148/433 |
| 5,002,732 | 3/1991  | Yamasaki et al.  | 420/473 |

#### OTHER PUBLICATIONS

Patent Abstracts of Japan Pub. No. 03002341. Appl. Date 5/26/89 Appl. No. 01133378, Jan. 8, 1991.

Abstract of Japanese Document No. JP06184678, Sep. 21, 1994.

Abstract of Japanese Document No. JP63161134, Sep. 23, 1993.

Abstract of Japanese Document No. JP62182240, Sep. 22, 1993.

Abstract of Japanese Document No. JP06220594, Nov. 2, 1994.

*Primary Examiner*—John Sheehan

*Attorney, Agent, or Firm*—Bachman & LaPointe, P.C.

### [57] ABSTRACT

A copper base alloy consisting essentially of tin in an amount from about 0.1 to about 1.5% by weight phosphorous in an amount from about 0.01 to about 0.35% by weight, iron in an amount from about 0.01 to about 0.8% by weight, zinc in an amount from about 1.0 to about 15% by weight, and the balance essentially copper, including phosphide particles uniformly distributed throughout the matrix, is described. The alloy is characterized by an excellent combination of physical properties. The process of forming the copper base alloy described herein includes casting, homogenizing, rolling, process annealing and stress relief annealing.

**10 Claims, No Drawings**

## COPPER ALLOY AND PROCESS FOR OBTAINING SAME

### CROSS-REFERENCE TO RELATED APPLICATION(S)

The present application is related to U.S. patent application Ser. No. 08/747,014, filed Nov. 7, 1996, entitled COPPER ALLOY AND PROCESS FOR OBTAINING SAME and to U.S. patent application Ser. No. 08/780 116, filed Dec. 26, 1996, entitled COPPER ALLOY AND PROCESS FOR OBTAINING SAME.

### BACKGROUND OF THE INVENTION

The present invention relates to copper base alloys having utility in electrical applications and to a process for producing said copper base alloys.

There are a number of copper base alloys that are used in connector, lead frame and other electrical applications because their special properties are well suited for these applications. Despite the existence of these alloys, there remains a need for copper base alloys that can be used in applications that require high yield strength greater than 80 KSI, together with good forming properties that allow one to make 180° badway bends with a R/T ratio of 1 or less plus low relaxation of stress at elevated temperatures and freedom of stress corrosion cracking. Alloys presently available do not meet all of these requirements or have high costs that make them less economical in the marketplace or have other significant drawbacks. It remains highly desirable to develop a copper base alloy satisfying the foregoing goals.

Beryllium copper generally has very high strength and conductivity along with good stress relaxation characteristics; however, these materials are limited in their forming ability. One such limitation is the difficulty with 180° badway bends. In addition, they are very expensive and often require extra heat treatment after preparation of a desired part. Naturally, this adds even further to the cost.

Phosphor bronze materials are inexpensive alloys with good strength and excellent forming properties. They are widely used in the electronic and telecommunications industries. However, they tend to be undesirable where they are required to conduct very high current under very high temperature conditions, for example under conditions found in automotive applications for use under the hood. This combined with their high thermal stress relaxation rate makes these materials less suitable for many applications.

High copper, high conductivity alloys also have many desirable properties, but generally do not have mechanical strength desired for numerous applications. Typical ones of these alloys include, but are not limited to, copper alloys 110, 122, 192 and 194.

Representative prior art patents include U.S. Pat. Nos. 4,666,667, 4,627,960, 2,062,427, 4,605,532, 4,586,967, 4,822,562, and 4,935,076.

Accordingly, it is highly desirable to develop copper base alloys having a combination of desirable properties making them eminently suitable for many applications.

### SUMMARY OF THE INVENTION

In accordance with the present invention, it has been found that the foregoing objective is readily obtained.

Copper base alloys in accordance with the present invention consist essentially of tin in an amount from about 0.1 to about 1.5%, preferably from about 0.4 to 0.9%, phosphorous

in an amount from about 0.01 to about 0.35%, preferably from about 0.1% to about 0.1%, iron in an amount from about 0.01% to about 0.8% preferably from about 0.05% to about 0.25% zinc in an amount from about 1.0 to about 15%, preferably from about 6.0 to about 12.0%, and the balance essentially copper. It is particularly advantageous to include nickel and/or cobalt in an amount up to about 0.5% each, preferably in an amount from about 0.001% to about 0.5% each. Alloys in accordance with the present invention may also include up to 0.1% each of aluminum, silver, boron, beryllium, calcium, chromium, indium, lithium, magnesium, manganese, lead, silicon, antimony, titanium, and zirconium. As used herein, the percentages are weight percentages.

It is desirable and advantageous in the alloys of the present invention to provide phosphide particles of iron and/or nickel and/or magnesium or a combination thereof, uniformly distributed throughout the matrix since these particles serve to increase strengths conductivity, and stress relaxation characteristics of the alloys. The phosphide particles may have a particle size of 50 Angstroms to about 0.5 microns and may include a finer component and a coarser component. The finer component may have a particle size ranging from about 50 to 250 Angstroms, preferably from about 50 to 200 Angstroms. The coarser component may have a particle size generally from 0.075 to 0.5 microns, preferably from 0.075 to 0.125 microns.

The alloys of the present invention enjoy a variety of excellent properties making them eminently suitable for use as connectors, lead frames, springs and other electrical applications. The alloys should have an excellent and unusual combination of mechanical strength, formability, thermal and electrical conductivities, and stress relaxation properties.

The process of the present invention comprises: casting a copper base alloy having a composition as aforesaid; homogenizing at least once for at least one hour at temperatures from about 1000 to 1450° F.; rolling to finish gauge including at least one process anneal for at least one hour at 650 to 1200° F.; and stress relief annealing for at least one hour at a temperature in the range of 300 to 600° F., thereby obtaining a copper alloy including phosphide particles uniformly distributed throughout the matrix. Nickel and/or cobalt may be included in the alloy as above.

### DETAILED DESCRIPTION OF THE PREFERRED EMBODIMENT(S)

The alloys of the present invention are modified copper-tin-zinc alloys. They are characterized by higher strengths, better forming properties, higher conductivity, and stress relaxation properties that represent a significant improvement over the same properties of the unmodified alloys.

The alloys in accordance with the present invention include those copper base alloys consisting essentially of tin in an amount from about 0.1 to 1.5%, preferably from about 0.4 to about 0.9%, phosphorous in an amount from about 0.01 to about 0.35%, preferably from about 0.01 to about 0.1%, iron in an amount from about 0.01 to about 0.8%, preferably from about 0.05 to about 0.25%, zinc in an amount from about 1.0 to about 15%, preferably from about 6.0 to about 12.0%, and the balance essentially copper. These alloys typically will have phosphide particles uniformly distributed throughout the matrix.

These alloys may also include nickel and/or cobalt in an amount up to about 0.5% each, preferably from about 0.001 to about 0.5% of one or combinations of both.

One may include one or more of the following elements in the alloy combination: aluminum, silver, boron, beryllium, calcium, chromium, indium, lithium magnesium, manganese lead, silicone antimony, titanium, and zirconium. These materials may be included in amounts less than 0.1%, each generally in excess of 0.001 each. The use of one or more of these materials improves the mechanical properties such as stress relaxation properties; however, larger amounts may affect conductivity and forming properties.

The aforesaid phosphorous addition allows the metal to stay deoxidized making it possible to cast sound metal within the limits set for phosphorous, and with thermal treatment of the alloys, phosphorous forms a phosphide with iron and/or iron and nickel and/or iron and magnesium and/or a combination of these elements if present, which significantly reduces the loss in conductivity that would result if these materials were entirely in solid solution in the matrix. It is particularly desirable to provide iron phosphide particles uniformly distributed throughout the matrix as these help improve the stress relaxation properties by blocking dislocation movement.

Iron in the range of about 0.01 to about 0.8% and particularly about 0.05 to about 0.25% increases the strength of the alloys, promotes a fine grain structure by acting as a grain growth inhibitor and in combination with phosphorous in this range helps improve the stress relaxation properties without negative effect on electrical and thermal conductivities.

Nickel and/or cobalt in an amount from about 0.001 to 0.5% each are desirable additives since they improve stress relaxation properties and strength by refining the grain and through distribution throughout the matrix, with a positive effect on the conductivity.

The process of the present invention includes casting an alloy having a composition as aforesaid. Any suitable casting technique known in the art such as horizontal continuous casting may be used to form a strip having a thickness in the range of from about 0.500 to 0.750 inches. The processing includes at least one homogenization for at least one hour, and preferably for a time period in the range of from about 1 to about 24 hours, at temperatures in the range of from about 1000 to 1450° F. At least one homogenization step may be conducted after a rolling step. After homogenization, the strip may be milled once or twice to remove from about 0.020 to 0.100 inches of material from each face.

The material is then rolled to final gauge including at least one process anneal at 650 to 1200° F. for at least one hour and preferably for about 1 to 24 hours, followed by slow cooling to ambient at 20 to 200° F. per hour.

The material is then stress relief annealed at final gauge at a temperature in the range of 300 to 600° F. for at least one hour and preferably for a time period in the range of about 1 to 20 hours. This advantageously improves formability and stress relaxation properties.

The thermal treatments advantageously and most desirably provide the alloys of the present invention with phosphide particles of iron and/or nickel and/or magnesium or a combination thereof uniformly distributed throughout the matrix. The phosphide particles increase the strength, conductivity, and stress relaxation characteristics of the alloys. The phosphide particles may have a particle size of about 50 Angstroms to about 0.5 microns and may include a finer component and a coarser component. The finer component may have a particle size of about 50 to 250 Angstroms preferably from about 50 to 200 Angstroms. The coarser component may have a particle size generally from 0.075 to 0.5 microns, preferably from 0.075 to 0.125 microns.

Alloys formed in accordance with the process of the present invention and having the aforesaid compositions are capable of achieving a yield strength in the 80–10 ksi range with bending ability at a radius equal to its thickness. 5 badwaye on a width up to 10 times the thickness. Additionally, they are capable of achieving an electrical conductivity of the order of 35% IACS, or better. The foregoing coupled with the desired metallurgical structure should give the alloys a high stress retention ability, for 10 example over 60% at 150° C., after 1000 hours with a stress equal to 75% of its yield strength on samples cut parallel to the direction of rolling, and makes these alloys very suitable for a wide variety of applications requiring high stress retention capabilities. Moreover, the present alloys do not 15 require further treatment by stampers.

This invention may be embodied in other forms or carried out in other ways without departing from the spirit or essential characteristics thereof. The present embodiments are therefore to be considered as in all respects illustrative 20 and not restrictive, the scope of the invention being indicated by the appended claims, and all changes which come within the meaning and range of equivalency are intended to be embraced therein.

What is claimed is:

25 1. A process for preparing a copper base alloy which comprises: casting a copper base alloy consisting essentially of tin in an amount from about 0.1 to about 1.5% by weight, phosphorous in an amount from about 0.01 to about 0.35% by weight, iron in an amount from about 0.01 to about 0.8% 30 by weight, zinc in an amount from about 1.0 to about 15% by weight, and the balance essentially copper; homogenizing at least once for at least one hour at a temperature from 1000 to 1450° F.; rolling to final gauge including at least one process anneal for at least one hour at 650 to 1200° F. 35 followed by slow cooling; and stress relief annealing at final gauge for at least one hour at 300 to 600° F., thereby obtaining a copper base alloy including phosphide particles uniformly distributed throughout.

2. Process according to claim 1, wherein said copper base 40 alloy being cast includes a material selected from the group consisting of nickel, cobalt and mixtures thereof in an amount from about 0.001 to about 0.5% each.

3. Process according to claim 2, wherein said copper base 45 alloy being cast includes magnesium and said phosphide particles are selected from the group consisting of iron nickel phosphide particles, iron magnesium phosphide particles, iron phosphide particles, magnesium nickel phosphide particles, magnesium phosphide and mixtures thereof.

4. Process according to claim 3, wherein said phosphide 50 particles have a particle size of from 50 Angstroms to 0.5 microns.

5. Process according to claim 1, including two homogenization steps, wherein at least one homogenization step is 55 subsequent to a rolling step and wherein the homogenization steps are for 2 to 24 hours each.

6. Process according to claim 1, wherein said process anneal is for 1 to 24 hours.

7. Process according to claim 1, wherein said stress relief 60 anneal is for 1 to 20 hours.

8. Process according to claim 1, wherein said casting step forms a strip having a thickness from 0.500 to 0.750 inches and said process further includes milling said strip at least once following said homogenizing step.

9. Process according to claim 1, wherein said cooling step 65 is performed at a cooling rate of 20 to 200° F. per hour.

10. A process for preparing a copper base alloy which comprises: casting a copper base alloy consisting essentially

of tin in an amount from about 0.4 to about 0.9% by weight, zinc in an amount from about 6.0 to about 12.0% by weight, phosphorous in an amount from about 0.01 to about 0.2% by weight, iron in an amount from about 0.01 to about 0.8% by weight, a material selected from the group consisting of nickel, cobalt and mixtures thereof in an amount from about 0.001 to about 0.5% by weight each, and the balance essentially copper; homogenizing at least once for at least one hour at a temperature from 1000 to 1450° F; rolling to

final gauge including at least one process anneal for at least one hour at 650 to 1200° F, followed by slow cooling; and stress relief annealing at final gauge for at least one hour at 300 to 600° F, thereby obtaining a copper base alloy including phosphide particles uniformly distributed throughout.

\* \* \* \* \*